

# UNITED STATES PATENT OFFICE.

FREDERICK W. HOCHSTETTER, OF NEW YORK, N. Y., ASSIGNOR TO PAUL M. PIERSON,  
OF SCARBORO-ON-THE-HUDSON, NEW YORK.

## RESTORATIVE FOR BLEMISHED MOVING-PICTURE FILMS.

1,139,680.

Specification of Letters Patent. Patented May 18, 1915.

No Drawing.

Application filed May 27, 1913. Serial No. 770,177.

*To all whom it may concern:*

Be it known that I, FREDERICK W. HOCHSTETTER, a subject of the Emperor of Germany, and a resident of New York, county 5 and State of New York, have invented a certain new and useful Restorative for Blemished Moving-Picture Films, of which the following is a full, clear, and exact specification.

This invention relates to a modified composition of matter disclosed in my pending application for Letters Patent, serially numbered 732,465, and filed November 20, 1912.

In accordance with present methods in practice it is customary in exhibiting moving pictures to transmit the transparent film through a kinetoscope for projecting the pictures thereof upon a curtain, or screen. The film being of a peculiar composition 20 makes it susceptible of attracting dust, or the like as it is directed through the mechanism, and the photography of the pictures on the film thereby becomes blemished by scratches, which produce "flickers" in the 25 pictures when projected, and moreover the pressure to which the film is subjected causes it to become hard and brittle.

My invention has for its object to overcome these objections by providing a composition of matter designed to be applied upon moving picture films when blemished in this manner by being adapted to remove 30 from the crevices of the scratches the dust settled therein, and which tends to restore 35 the transparency of the photography of the pictures by clearing the high lights and shadows thereof of all foreign substances as well as serving to restore the flexibility of the film.

This composition of matter consists of the following ingredients, combined in the proportions stated, viz:—a fatty base, such as tallow, lard, bees wax, paraffin, spermaceti, or the like 6 ounces; gum camphor, 5 drams; 40 alcohol, (U. S. P. strength) by weight, 2 ounces; sulfuric ether, (U. S. P. strength) by weight,  $\frac{1}{2}$  ounce; glycerin, by weight, 1 ounce.

The gum camphor is first dissolved in a

suitable container in the alcohol, and the fatty base is then melted in a separate vessel at a moderate temperature. When the fatty base is in a melted state the glycerin is added thereto and the ingredients are thoroughly mingled in any suitable manner. 55 The solution of camphor and the sulfuric ether are then mixed together, and after the mixture of the glycerin and fatty base has sufficiently cooled this solution is incorporated therewith by agitation through the use 60 of any desired method whereby a uniform emulsion is produced.

In using my composition for restoring moving picture films when impaired, as above described, a quantity of the emulsion 65 is applied by any suitable means to form a coating upon the film, and sufficient friction is employed to cause the emulsion to penetrate the crevices of the scratches therein as well as softening the texture of the 70 film. By the use of a pad, or buffer the excess of the coating of emulsion is removed from the film which in turn will free the scratches and the pictures of all particles of dust and foreign substances so that the normal clearness of the pictures will to a large 75 extent be renewed, and the flexibility of the film will also be restored.

Having thus described my invention, I claim as new and desire to secure by Letters Patent:—

1. The herein described restorative for blemished moving picture films comprising in combination, a fatty base, camphor, alcohol, sulfuric ether, and glycerin, substantially as set forth.

2. The herein described restorative for moving picture films comprising in the following proportions, a fatty base six ounces, camphor five drams, alcohol two ounces, sulfuric ether one-half ounce, and glycerin one ounce, substantially as described.

This specification signed and witnessed this twenty-sixth day of May, A. D. 1913.

FREDERICK W. HOCHSTETTER.

Witnesses:

ROBT. B. ABBOTT,  
M. DERMODY.